

## UNITED STATES PATENT OFFICE

2,290,549

## PROCESS FOR THE SEPARATION AND RECOVERY OF METALS FROM METALLIC ALLOYS

John D. Gat, Edgewood, Pa.

No Drawing. Application December 3, 1940,  
Serial No. 368,389

2 Claims. (Cl. 75—64)

This invention relates to the separation and recovery, in pure metallic state, of one of the elementary constituents of certain binary metallic alloys. The development relates particularly to the treatment of waste products of tin plate industry and to recovery of tin from such by-products of tin smelting practice as hard-head.

During the manufacture of tin plate, the pots must be frequently cleaned from heavy metal, iron-tin compounds which have settled to the bottom, and from a suspension of tin oxide and metallic tin in palm oil floating on the top and known as scruff. This operation, technically termed dressing, removes heavy metal together with comparatively large amounts of tin held by capillary attraction among the crystals of the iron-tin compound. The tin so removed is recovered by heating this heavy metal in sweating furnaces so as to cause liquation. This treatment oxidizes the solid body of iron-tin compounds to some extent.

As the scruff so removed carries large amounts of palm oil, the inorganic constituents of it must be separated from the palm oil by burning the latter off in the same furnaces as used for liquating heavy metal. The residues remaining in the sweating furnaces after liquation and after burning off, both of which are somewhat oxidized, are combined, as a rule, producing so-called tin dross which must be then subjected to special treatments for the recovery of tin.

The advantages of my process may best be understood by a brief consideration of the prior practices employed to recover tin from tin-iron alloys, either as a pure metal or as some suitable alloy.

Purely metallurgical methods proposed and used until now for the recovery of tin from these alloys do not give a direct solution of the problem and achieve the desired results in a somewhat roundabout manner.

When the iron concentration of the alloys is comparatively low, the element is separated from tin either by liquation or by segregation. In the methods involving liquation, the alloy, cast in blocks, is heated slightly above the melting point of pure tin but considerably below the temperature at which the iron-tin intermetallic compounds begin to melt. Molten tin flows from the solid framework of the latter and is separated from it. In the segregation methods, the alloys of iron and tin are melted in reverberatory furnaces and then slowly cooled, until a crust of iron-tin compounds is formed on the top of the

bath, after which the liquid tin is tapped from beneath the crust.

These methods cannot be applied, however, to iron-rich tin alloys. In the processes of the prior art, alloys belonging to this category were either returned, as a part of charge, to the tin-melting furnaces, when hardhead had to be disposed of, or melted in the presence of lead, which dissolves tin in all proportions without dissolving any iron, a practice common to the tin plate industry. The first method involves an elaborate plant and removes only a portion of iron by transforming it into silicates. Reduction in the presence of lead results in a tin-lead alloy containing about 20 percent tin; so that the utilization of the metal so produced is limited to terne coating and similar applications only. The process of my invention permits the recovery of tin in a pure state, even from high iron alloys.

10 The fundamental principles of my invention were discovered during the course of my efforts to develop an improved process for separating tin from iron contained in the tin-iron alloys. I have found that the problem can be effectively and 15 economically solved by introducing, under proper conditions, aluminum in the iron-tin system. Aluminum alloys both with iron and tin in any proportions, provided the temperature is sufficiently high, and forms, on cooling, intermetallic 20 compounds with the iron which are more stable than the intermetallic compounds of the latter with tin, so that iron-tin compounds cannot form in the presence of an excess of aluminum. The Fe<sub>2</sub>Al<sub>3</sub> so produced has a high melting point and 25 a low specific gravity, as compared with tin. Any excess of aluminum present in the system above that required for formation of iron compounds, precipitates from the system on cooling, having a very low solubility in tin near the melting point of the latter, and rises to the surface. 30 These characteristics permit both a complete elimination of the iron and of the aluminum which has been introduced for the removal of the former from the tin.

35 According to my invention, iron is separated from tin in the following manner. The iron-tin alloy to be treated is completely liquefied by heating it to a sufficiently high temperature, either with or without protection exerted by a suitably chosen cover of slag or any other appropriate substance. A sufficient amount of aluminum is added to the liquid bath to convert all iron present into Fe<sub>2</sub>Al<sub>3</sub>, allowing for a slight excess required for keeping the iron-tin compounds from forming. After aluminum is thoroughly incor-

porated, the bath is cooled below the solubility point of  $Fe_2Al_3$ , but above the melting point of tin, and is held at this temperature long enough to permit upward settling of the desired amount of the iron-bearing compounds. Instead of keeping the melt at a given temperature, it may be allowed to cool continuously at a sufficiently slow rate. The crust of the iron-aluminum alloy formed in this way is separated from the body of the underlying tin. This separation can be made before a complete separation is effected. In this case, the impure tin removed from under the crust is held just above its melting point long enough to permit all iron-bearing compounds and any possible excess of aluminum to rise to the surface, from which they are mechanically removed. The length of time required for this separation treatment depends on the degree of the desired purity of tin.

In order to adjust the process to optimum efficiency under the conditions existing in tin plate industry, I prefer to charge both heavy metal and scuff directly in a shaft furnace, a cupola, for example, together with some proper reducing material, such as coke, reduce tin oxides by keeping a strongly reducing atmosphere, melt tin and tin-iron alloys, keeping temperature sufficiently high to volatilize all zinc, tap the metal in an appropriate container, add to it a sufficiency of aluminum to combine with all iron and to leave a slight excess, cool the liquid alloy until a heavy crust of solid iron-aluminum alloy is formed on its surface, separate from it the body of still liquid tin underlying it by proper means and free this tin from the last traces of iron and aluminum by holding the metal at a temperature slightly above its melting point and mechanically removing from its surface solid phases rising to it, the use of some protecting cover, such as palm oil, being optional during the last operation.

It is well known that, for many metallurgical processes, the use of aluminum-iron alloys is preferable to the introduction of commercially pure aluminum. However, the general adoption of this practice in steel plants heretofore has been handicapped by the costs involved in the preparation of such alloys. I have discovered that the ferro-aluminum alloy produced by the processes of the present invention eliminates this handicap and offers an improved deoxidizing agent for the deoxidization of steel.

I claim:

1. A process for separating tin from an iron-tin alloy, including heating the alloy to render it liquid, adding aluminum to the liquid to produce an iron-aluminum compound dissolved in tin, cooling the liquid to a temperature below the solubility point of the compound in the tin, but substantially above the melting point of the tin, holding the liquid at this temperature until a portion of the compound separates from the liquid tin, removing this portion from the liquid tin, further cooling the liquid to a temperature just slightly above the melting point of tin, so that the remainder of the compound separates from the tin, and removing this remainder from the tin.
2. A process for separating tin from an iron-tin alloy, including heating the alloy to render it liquid, adding aluminum to the liquid to produce an iron-aluminum compound dissolved in tin, cooling the liquid to a temperature below the solubility point of the compound in the tin, but above the melting point of the tin, and separating the tin from the compound, the alloy initially containing oxides being heated to render it liquid while under conditions causing reduction of these oxides.